

Dec. 8, 1942.

W. H. GERISCH

2,304,561

LIQUID CONTACT CIRCUIT CLOSER

Filed Jan. 7, 1941

Fig. 3



Fig. 4



Fig. 2



Fig. 1



Fig. 5



Fig. 6



Fig. 7



INVENTOR

WALTER H. GERISCH.

BY

Harry E. Dunham

ATTORNEY

## UNITED STATES PATENT OFFICE

2,304,561

## LIQUID CONTACT CIRCUIT CLOSER

Walter H. Gerisch, North Bergen, N. J., assignor  
to General Electric Company, a corporation of  
New York

Application January 7, 1941, Serial No. 373,440

11 Claims. (Cl. 200—152)

The present invention relates to liquid-contact circuit closers of the type having an envelope containing a small quantity of mercury which is arranged to complete and interrupt the circuit between the terminals of the circuit closer. The invention is particularly concerned with circuit closers of the type in which the major portion of the envelope is constituted of two terminal-forming parts which are joined peripherally by a body of glass and which are separated within the envelope by an apertured ceramic barrier adapted to perform a circuit-interrupting function.

It is a primary object of the invention to provide an improved construction for liquid-contact circuit closers of the type above specified and more particularly to increase the safe current-carrying capacity of such circuit closers of the type above specified and more particularly to increase the safe current-carrying capacity of such circuit closers. In this connection a principal feature of the invention consists in improvements in the structure and composition of the circuit-interrupting barriers employed.

For a consideration of what I believe to be novel and my invention, attention is directed to the accompanying description and the claims appended thereto.

In the accompanying drawing:

Fig. 1 is a sectional elevation of a liquid contact circuit closer embodying my invention;

Fig. 2 is a sectional view taken on line 2—2 of Fig. 1;

Fig. 3 is a sectional elevation of a modification;

Fig. 4 is a sectional view on line 4—4 of Fig. 3;

Fig. 5 is a sectional elevation of another modification, and

Figs. 6 and 7 are sectional views of a still further modification.

Each of the circuit closers illustrated in Figs. 1 to 6, inclusive, has an envelope 1 containing a limited quantity of mercury 2. The major portion of the envelope comprises opposed straight-drawn cup-shaped metal terminals 3 juxtaposed to form an enclosed space between them. Between the terminals is a diaphragm or barrier 4 or 9 of insulating material having an opening 5 therein through which the mercury flows in order to complete a circuit between the terminals 3, 3. When the said circuit closers are in the position illustrated, the circuit between the terminals is complete. The members 3, 3 are hermetically joined by means of a thin ring 6 of glass or other thermo-plastic material sealed directly thereto in such a way as to be also in con-

tinuous contact with the outer periphery of the diaphragm 4.

When the circuit closers of Figs. 1 to 5, inclusive, are rotated about the axis of symmetry of the terminals a few degrees from the position illustrated, the opening 5 is raised clear of the mercury, and the circuit between the terminals is broken by separation of the mercury within the opening as it flows from each end thereof. 10 In this position, the diaphragm separates the mercury into two pools. When the circuit closer is returned to the position illustrated, the circuit between the terminals is completed by the joining of mercury flowing into the opening 5 from each end thereof.

It is not necessary in all cases that the circuit closers shall be rotated about the axis of symmetry of the terminals as described in connection with Figs. 1 to 5. In some cases, it is advantageous that the break in the mercury shall be brought about by tilting the circuit closer as shown in Figs. 6 and 7, in which event the opening 5 is preferably located at the center of the diaphragm, and sufficient mercury is provided to insure the closing of the circuit when the circuit closer is in an upright position. With the circuit closer in the position shown in Fig. 6, tilting the circuit closer to the left, for example a few degrees from the vertical, as shown in Fig. 7, causes the mercury above the right hand edge of the opening 5 to flow to the opposite side of the diaphragm, the portion of the mercury on the side of the barrier below the said edge being retained there, and the circuit between the terminals is broken by separation of the mercury at the said edge as it flows from the opening 5. In this position, the diaphragm separates the mercury into two pools. When the circuit closer is returned to the position illustrated in Fig. 6, the circuit between the terminals is completed by the joining of the said mercury pools by the mercury flowing back into the opening 5.

A charge of hydrogen ranging in pressure from about 1 atmosphere to much higher pressures 45 may advantageously be employed in connection with a switch such as that illustrated. Such hydrogen may be introduced into the switch during the manufacturing process through an opening 7, provided in the metal member 3. This opening 7 is thereafter sealed, preferably by fusion welding a closure member 8 therein, for example, in accordance with the procedure described and claimed in John H. Payne Patent 2,141,932, issued December 27, 1938.

Successful operation of circuit closers of the

type under consideration requires that the enclosing envelope be completely gas tight. In a construction such as that shown in Fig. 1, the fulfillment of this condition is complicated by the fact that the glass closure element 6 must be capable of sealing not only to the metal terminals 3 but also to the ceramic barrier 4. The successful matching of these diverse elements is a matter of considerable difficulty.

In circuit closers of this type heretofore commercially available good results have been obtained by forming the metal parts 3 of a chrome iron alloy and the glass sealing ring 6 of a relatively high expansion glass capable of sealing to such an alloy. In this latter connection it has proven desirable to use a lead glass having an expansivity on the order of  $9 \times 10^{-6}$  centimeters per centimeter per degree centigrade, this expansivity being provided, for example, by a glass having a composition within the following range:

|                  | Per cent  |
|------------------|-----------|
| PbO              | 20-30     |
| Alkali oxide     | 10-16     |
| SiO <sub>2</sub> | Remainder |

One example of such a glass is that sold by the Corning Glass Company under the code Number 001.

In order that the ceramic barrier may sufficiently match the sealing glass to avoid producing excessive strains in it, it has been found expedient to form it of magnesia (a material of very high expansivity) in combination with a vitreous bonding substance, such as clay, which is characterized by low expansivity, the materials being admixed in proportions calculated to reduce the expansivity of the composition as a whole to a value commensurate with that of the sealing glass. Barriers of this type are described and claimed in Louis Navias Patent 2,153,000, issued April 4, 1939.

Circuit closers of the construction just specified have functioned successfully in practice and have been sold extensively for low current use. In attempting to extend their application to high current circuits, however, certain difficulties are encountered. In particular it is found that there is a tendency for excessive erosion of the ceramic barrier to occur if the circuit closer is used to control currents greater than a few amperes.

In accordance with the present invention this limitation is substantially overcome by incorporating in the barrier, either superficially or throughout its structure, a quantity of a glass of the low expansion borosilicate type. In the preferred case a ceramic of the desired quality is prepared by fusing a mixture of a granular refractory material having a high coefficient of expansion (e.g. magnesia) and a vitrifiable binder including a substantial amount of a glass of the above-specified type, the relative proportions of the combined materials being adjusted to produce a coefficient of expansion of the ceramic as a whole which is matched to that of the sealing glass by which the metallic envelope parts are joined. In this connection it is to be noted that while typical borosilicate glasses have expansion coefficients on the order of  $3 \times 10^{-6}$  centimeters per centimeter, magnesia has an expansion coefficient above  $14 \times 10^{-6}$ . Consequently, a substantial quantity of borosilicate glass may be combined with magnesia without producing a resultant expansivity too low for proper cooperation with the sealing glass.

In particular I have found that a ceramic hav-

ing a coefficient of expansion sufficiently close to that of a lead sealing glass such as Corning 001 may be produced by combining powdered fused magnesia with clay and with a glass of the Pyrex type. For the latter constituent one may use, for example, a borosilicate glass having approximately the following oxide composition:

|                                | Per cent |
|--------------------------------|----------|
| SiO <sub>2</sub>               | 80.5     |
| B <sub>2</sub> O <sub>3</sub>  | 12.9     |
| Na <sub>2</sub> O              | 3.8      |
| K <sub>2</sub> O               | 0.4      |
| Al <sub>2</sub> O <sub>3</sub> | 2.2      |
|                                | 99.8     |

This is a typical analysis of the glass sold by the Corning Glass Company under their code No. 774.

20 The composition of the ceramic may be varied within limits approximately as follows:

|          | Per cent  |
|----------|-----------|
| Magnesia | 65-75     |
| Glass    | 5-20      |
| Clay     | Remainder |

A particular mixture which I have found to have the desired properties consists of

|               | Per cent |
|---------------|----------|
| Magnesia      | 75       |
| Ball clay     | 15       |
| No. 774 glass | 10       |

In combining the materials the clay is first added to the magnesia, both of these being preferably powdered to 200 mesh fineness. Thorough admixture of the ingredients is secured by tumbling them for approximately two hours in a ball mill. To render this combination readily moldable one may add a few percent of a temporary binder such, for example, as paraffin wax heated to its melting point. The batch is then transferred to a dough mixer and heated to the melting temperature of the wax, whereupon the hot liquid wax is added to the batch and the

45 mass is kneaded until the batch has cooled down to room temperature. Thereafter dry powdered borosilicate glass of 200 mesh fineness is added and the batch is further kneaded for 15 or 20 minutes to insure thorough dispersal of the glass powder through the batch. Portions of this composition may be placed in molds of desired shape and size and exposed to a sufficient degree of pressure to assure a compactly molded product.

50 Thereafter the molded articles are fired at a temperature of between 1100° and 1200° C. (preferably about 1150° C.) to remove the temporary binder and to vitrify and fuse the clay and glass ingredients, thus binding all the parts together. A firing time of as little as three minutes at

60 1150° C. has been found to be sufficient to produce a highly durable, hard, uniform and non-porous product.

65 Barriers constituted as described in the foregoing are capable of being sealed in place in a circuit closer of the type under consideration without cracking the sealing glass by which the metal parts of the device are joined, this result being a consequence of the correlation of the expansivity of the ceramic with the corresponding property of the sealing glass. In addition, due to the presence of the borosilicate glass component, such barriers are highly resistant to heat shock and to the erosive action of arcs formed during circuit making and breaking operations.

70 75 The improvement in this latter respect over oth-

erwise similar barriers in which the glass constituent is omitted is so great as to double the current which may be interrupted by a given form of barrier without excessive erosion of the barrier surfaces.

The advantages realized from the use of the improved ceramic compositions specified in the foregoing which make them useful in the arts generally and particularly as electrical insulators, are still further enhanced by providing each of the barrier elements with a shoulder which projects outwardly from the barrier at least in the region between the barrier opening and the most nearly adjacent portion of the envelope wall. Such a shoulder, which is exemplified in Fig. 1 as a continuous flange 11, is preferably formed so that its inner surface in the region between the barrier opening and the most nearly adjacent part of the envelope wall comprises a rectilinear extension of the surface by which such opening is internally bounded. As so formed, its utility is considered to be due to the fact that it serves to prevent the arc formed during a circuit making or breaking operation from becoming terminally attached to the envelope wall near the glass-to-metal seal, thus creating a danger of cracking the seal. Furthermore, the combination of such a shoulder with the straight-drawn envelope construction shown is found to prevent repetitive attachment of the arc to any particular point on the envelope wall surface, and for this reason localized overheating and puncturing of the envelope are avoided.

Results generally similar to those described above as being attributable to the incorporation of boro-silicate glass in the ceramic structure may also be obtained by the application of a coating of this glass to the surface of a barrier 9 which is otherwise constituted principally of magnesia and clay, such a coating being indicated at 10 in Fig. 3. In this embodiment, which is somewhat more difficult to fabricate than that previously described, the glass coating must be extremely thin in order to avoid cracking due to the expansion differences between the glass and the ceramic. However, if a thickness on the order of a few mils is employed, there is little tendency for the glass coating to become separated from the ceramic as a result of expansion differences, and the erosion-resisting properties of the coated surfaces are very greatly improved, making the structures useful in the arts generally and particularly as electrical insulators. Insulators of the composition specified are further described and claimed in my copending application Serial No. 423,413, filed December 18, 1941, and assigned to the same assignee as the present application.

In the construction of Figs. 3 and 4 as in that of Fig. 1, the ceramic barrier is advantageously provided with a projecting shoulder adapted to protect the adjacent surfaces of the envelope from the action of the arc formed during the use of the circuit closer. In this case, however, the shoulder which is indicated at 12 does not extend continuously around the circumference of the barrier but is limited to the particular region in which the action of the arc tends to be most pronounced.

Fig. 5 illustrates a further possible modification of the invention; namely, the combined use of a ceramic incorporating a quantity of borosilicate glass as an essential part of the ceramic composition and a coating 10 of such glass applied to the surface of the ceramic.

By the use of the improvements described in the foregoing it has proven possible to increase the current rating of a given switch as much as one hundred percent above the value previously considered safe without significantly changing the over-all dimensions of the switch. Moreover, this has been accomplished in a manner which does not add appreciably to the cost of the switch or increase the difficulties of its manufacture.

While the invention has been described by reference to particular embodiments thereof, it will be understood that numerous further modifications may be made by those skilled in the art without actually departing from the invention.

I, therefore, aim in the appended claims to cover all such equivalent variations and uses as come within the true spirit and scope of the foregoing disclosure.

What I claim as new and desire to secure by Letters Patent of the United States is:

1. A circuit closer of the type which comprises a multipart enclosure, a quantity of a liquid-contact medium within the enclosure, a quantity of sealing glass of relatively high expansivity joining the parts of the enclosure, and an apertured circuit-interrupting barrier within the said enclosure and sealed to the said glass, wherein the said barrier consists essentially of a high expansion refractory combined with a low expansion vitreous bonding material in such proportions as to produce a coefficient of expansion of the combination comparable to that of the said sealing glass and in which at least the circuit-interrupting surfaces of the barrier incorporate glass of the low expansion boro-silicate type.

2. A circuit closer of the type which comprises a multipart enclosure, a quantity of a liquid-contact medium within the enclosure, a quantity of sealing glass of relatively high expansivity joining the parts of the enclosure, and an apertured circuit-interrupting barrier within the said enclosure and sealed to the said glass wherein the said barrier consists essentially of magnesia and a vitreous bonding material containing a substantial proportion of a glass of the low expansion boro-silicate type, the magnesia and bonding material being combined in such proportions as to have a coefficient of expansion comparable to that of the said sealing glass.

3. A circuit closer of the type which comprises a multipart enclosure, a quantity of a liquid-contact medium within the enclosure, a quantity of sealing glass of relatively high expansivity joining the parts of the enclosure, and an apertured circuit-interrupting barrier within the said enclosure and sealed to the said glass, wherein the said barrier consists essentially of magnesia and a vitrified bonding material including at least 5% of a low expansion boro-silicate glass, said magnesia and said bonding material being combined in such proportions as to have a coefficient of expansion comparable to that of the sealing glass.

4. A circuit closer of the type which comprises a multipart enclosure, a quantity of a liquid-contact medium within the enclosure, a quantity of sealing glass of relatively high expansivity joining the parts of the enclosure, and an apertured circuit-interrupting barrier within the said enclosure and sealed to the said glass, wherein the said barrier consists essentially of magnesia, clay and a substantial quantity of glass of the low expansion borosilicate type, the magnesia, glass, and clay being combined in such propor-

tions as to have a coefficient of expansion comparable to that of the said sealing glass.

5. A circuit closer of the type which comprises a multipart enclosure, a quantity of a liquid-contact medium within the enclosure, a quantity of sealing glass of relatively high expansivity joining the parts of the enclosure, and an apertured circuit-interrupting barrier within the said enclosure and sealed to the said glass, wherein the said barrier consists essentially of magnesia combined with a low expansion vitreous bonding material in such proportions as to have a coefficient of expansion comparable to that of the said sealing glass and in which the circuit-interrupting surfaces of the barrier are coated with a thin layer of a glass of the low expansion boro-silicate type.

6. An interrupting element for a liquid-contact circuit closer, said element consisting essentially of a high expansion refractory and a low expansion vitreous bonding material including boro-silicate glass covering at least the circuit-interrupting surfaces of the element.

7. An interrupting element for a liquid-contact circuit closer, said element consisting essentially of fused magnesia and a low expansion vitreous bonding material including a substan-

tial proportion of a low expansion borosilicate glass.

8. An interrupting element for a liquid-contact circuit closer, said element consisting essentially of a high expansion refractory in combination with a low expansion vitreous bonding material and having the circuit interrupting surfaces of the element coated with a thin layer of low expansion boro-silicate glass.

10 9. An interrupting element for a liquid-contact circuit closer, said element consisting of a fused composition of from 65 to 75% fused magnesia, at least 5% of a low expansion borosilicate glass and a complementary proportion of clay.

15 10. An interrupting element for a liquid-contact circuit closer, said element consisting essentially of a composition of from 65 to 75% magnesia, from 5 to 20% of low expansion borosilicate glass and a complementary proportion of clay.

20 11. An interrupting element for a liquid-contact circuit closer, said element consisting essentially of about 75% magnesia, about 15% clay and about 10% of a low expansion borosilicate glass.

WALTER H. GERISCH.